

# United States Patent Office

2,917,160

Patented Dec. 15, 1959

1

2,917,160

## METAL WORKING METHOD AND LUBRICANT THEREFOR

Otto Turinsky, Western Spring, Ill., assignor to Armour and Company, Chicago, Ill., a corporation of Illinois

No Drawing, Application April 12, 1951  
Serial No. 220,707

6 Claims. (Cl. 205—2)

My invention relates to the working of metals, and particularly to the steps of applying a film of corrosion-inhibiting surface active lubricant to the surface of ferrous and non-ferrous metals and forming these metals by cutting, grinding or drawing methods.

An object of my invention is the provision of an economical method for cutting and drawing metals in a uniformly smooth manner without producing uneven surfaces and without causing a "ripping" effect.

Another object of my invention is the provision of a method of forming metals by the use of corrosion-inhibiting surface active lubricants.

Other objects of my invention will be apparent as this specification proceeds.

Many metal working operations such as drawing, grinding, cutting, etc. involve the common principle of contacting the surface of a metal part with a shaping tool or element so as to change the conformation or surface characteristics of the metal part. When such operations are carried out without the aid of lubricants, an undesirable amount of heat and friction is generated at the points of contact and a welding or binding effect is noted. Unless this heat can be dissipated, damage results to both the tool and the metal part, and in the case of poorly lubricated deep-drawing and pressure stamping there is the additional danger of fracturing the metal part.

It is well known that non-surface-active lubricants such as mineral oil are unsatisfactory for many metal working operations, especially the drawing of metals. Such lubricants have a tendency to flow away from the precise area in which the heat and pressure are greatest and where lubrication is most effective in preventing binding.

Emulsions of soap and fat in water have been used as cutting and drawing compounds. The degree of success attained with these compounds is due to the fact that soap, being surface active, adheres to the surface of the metal being processed as well as the surface of the shaping tool. Likewise soap has an affinity for fat which is thus held upon the surface of the metal in a lubricative film. However, fat and soap are unavoidably caustic in nature and as a result of their use the metal surface is soon corroded.

In general, a surface active compound is composed of a combination of a water-soluble or hydrophilic chemical group and an oil-soluble or hydrophobic chemical. If such a compound does not ionize, it is said to be non-ionic, while if it does ionize it is said to be ionic. When that part of the ionized molecule containing the oil-soluble portion is the positive ion, or cation, the compound is said to be cation-active or cationic. Those ionic compounds such as soap having an oil-soluble anion are known as anionic agents.

I have discovered that instead of using a soap-fat emulsion as a metal working lubricant I can use cationic tertiary amines to obtain excellent drawing and cutting characteristics while at the same time inhibiting corrosion of the metals.

2

Tertiary amines suitable for my process have the general formula.



where R is a long chain aliphatic hydrocarbon radical having 12 to 20 carbon atoms and where x and y are integral numbers from 1 to 49. For example, the long chain aliphatic radical R may be dodecyl, hexadecyl, eicosyl, octadecenyl, or octadecenyl. For my process I prefer to use N,N'-bis(2-hydroxy-ethyl) soya amine in which the soya radical comprises a mixture of saturated and unsaturated radicals including hexadecyl, octadecyl, octadecenyl, octadecenyl, and eicosyl. The number of ethenoxy groups as indicated by x and y may be varied. Thus, for five ethenoxy groups x and y may be 1 and 4 respectively or 2 and 3 respectively. Y may be greater than x, and the sum of x plus y may be as large as 50. In general, the water solubility of these hydroxylated tertiary amines is increased by the addition of ethenoxy groups. In my process I preferably use bis-(2-hydroxyethyl) aliphatic amines and their acid salts.

Although some of these hydroxylated tertiary amines as well as the hydroxylated tertiary amine acid salts are relatively insoluble in water, they may be employed in the form of an emulsion or saturated solution. For example, they may be used advantageously in a water emulsion in the ratio of one part of amine to 3 parts of water.

These amine compounds may be advantageously used in their water-soluble salt form. The amine salt is formed by contacting the amine with an acid. While the amine salts of strong acids may be used, I prefer to use the amine salts of weak acids. I use phosphoric acid with considerable advantage and in particular orthophosphoric acid. Some of the amine acid salts such as phosphoric and lactic are effective in inhibiting corrosion.

These hydroxylated tertiary amine salts are stable in aqueous solution below a pH of approximately 8. I have found that solutions of these salts are more effective as corrosion inhibitors above pH 5. Because of these limitations I prefer to practice my process using as a lubricant the acid salt of the amine in aqueous solution having a pH between about 5 and about 8.

The use of a solution of the hydroxylated tertiary amine salt of a weak acid is desirable for the reason that such a solution acts as a buffer and resists any change in the hydrogen-ion concentration on the addition of acid or alkali. This quality is important in a metal-working lubricant solution because during prolonged use the solution often becomes contaminated by small amounts of acid and alkali carried over from previous operations such as pickling, rinsing, etc.

A specific example of a formulation of a suitable drawing bath follows:

Approximately 300 grams of bis-(2-hydroxyethyl) soya amine are added to a liter of water. With constant stirring the amine is "solubilized" by adding a quantity of orthophosphoric acid sufficient to completely dissolve the amine in water. The pH of such a solution is approximately 7, and if desired the pH may be lowered by adding more phosphoric acid. The drawing bath is then made up by dissolving one part of this amine formulation in about forty parts of water.

In either a cutting or drawing operation, the surface of the metal to be formed may be immersed in an amine bath before passing to the forming elements such as drawing dies or cutting tools. If the metal stock cannot be conveniently immersed in the bath, the amine solution may be sprayed or poured on the metal surface be-

fore it is subjected to the forming step. Depending upon conditions encountered, the amine lubricant may be applied to the metal surface in dry form or in the form of a paste or solution. The method of applying the lubricant is not limited to immersion of the metal part, or spraying or pouring. In general any method of application is suitable which results in contacting the lubricant at the interface between the metal surface and the metal-working tool. Before passing to the metal working step a wet metal surface may first be allowed to dry without appreciably impairing the lubricative qualities. After the metal stock has been coated with a film of the amine lubricant, it may be processed with at least one forming tool before it is necessary to re-treat the surface with more lubricant. In some cases as many as three successive forming operations can be carried out without intermediate lubrication.

My process is not limited to the drawing or cutting of metals. In general, it may be practiced in any operation involving lubrication of the interface between a metal surface and a metal-working tool.

Other modifications of the process all within the spirit of my invention will readily occur to those skilled in the art.

I claim:

1. In the art of working metal by cutting, grinding, drawing, and the like, the step which comprises carrying out the process with the portions of the metal being worked in contact with a material selected from the group consisting of hydroxylated tertiary amines and the acid salts thereof, said amines having the general formula



wherein R is a straight chain aliphatic hydrocarbon radical having 12 to 20 carbon atoms and x and y are integral numbers, the sum of x and y being in the range from about 2 to 50.

2. In the art of working metal by cutting, grinding, drawing, and the like, the step which comprises carrying out the process with the portions of the metal being worked in contact with an aqueous solution containing approximately 3 parts by weight of water per part of an acid salt of a hydroxylated tertiary amine, said amine having the formula



wherein R is a straight chain aliphatic hydrocarbon radical having 12 to 20 carbon atoms and x and y are integral

10

numbers, the sum of x and y being in the range from about 2 to 50.

3. In the art of working metal by cutting, grinding, drawing, and the like, the step which comprises carrying out the process with the portions of the metal being worked in contact with an aqueous solution containing approximately 3 parts by weight of water per part of the phosphoric acid salt of a hydroxylated tertiary amine, said amine having the formula



15

wherein R is a straight chain aliphatic hydrocarbon radical having 12 to 20 carbon atoms and x and y are integral numbers, the sum of x and y being in the range from about 2 to 50.

4. A process according to claim 3 wherein the pH of said aqueous solution is in the range of from about 5 to about 8.

5. In a process for the drawing of metal, the step which comprises carrying out the process with the portions of the metal being drawn in contact with an aqueous solution containing approximately 3 parts by weight of water per part of the phosphoric acid salt of a hydroxylated tertiary amine having the formula



20

wherein R is a straight chain aliphatic hydrocarbon radical having 12 to 20 carbon atoms and x and y are integral numbers, the sum of x and y being in the range from about 2 to 50.

25

6. A process according to claim 1 wherein an acid salt of N - soya - bis(2 - hydroxypolyethoxyethyl) amine is employed.

#### References Cited in the file of this patent

#### UNITED STATES PATENTS

|           |                |                |
|-----------|----------------|----------------|
| 1,991,395 | Kocoor         | Oct. 24, 1932  |
| 2,223,037 | Ihrig          | Nov. 26, 1940  |
| 2,231,228 | Singer         | Feb. 11, 1941  |
| 2,233,383 | De Groot       | Feb. 25, 1941  |
| 2,275,198 | Patnode        | Mar. 3, 1942   |
| 2,297,221 | Huttenlocher   | Sept. 29, 1942 |
| 2,298,636 | Prutton        | Oct. 13, 1942  |
| 2,298,640 | Prutton        | Oct. 13, 1942  |
| 2,474,325 | Rodgers et al. | June 28, 1949  |
| 2,541,678 | Swanay         | Feb. 13, 1951  |